

# UNITED STATES PATENT OFFICE.

JAMES O. PERSONS, OF NORFOLK, VIRGINIA.

## NON-INFLAMMABLE WATERPROOFING COMPOSITION.

1,204,056.

Specification of Letters Patent.

Patented Nov. 7, 1916.

No Drawing.

Application filed April 26, 1915. Serial No. 24,144.

To all whom it may concern:

Be it known that I, JAMES O. PERSONS, a citizen of the United States, residing at Norfolk, in the county of Norfolk and State 5 of Virginia, have invented certain new and useful Improvements in Non-Inflammable Waterproofing Compositions; and I hereby declare that the following is a full, clear, and exact description thereof.

- 10 This invention relates to a new and improved water-proofing composition especially prepared for application to fabrics and the like, and has as an object to provide a water-proofing composition which is non-inflammable and which, when applied to fabrics and the like, renders the same non-inflammable, the composition and the fabric or material coated therewith being non-combustible.
- 15 It is a further object of this invention to provide a noninflammable water-proofing composition which may be easily applied and which will render the fabric to which it is applied impervious to water and moisture 20 by entering all the interstices therein.
- 25 Other characteristics of the composition are, that it is practically colorless and will not therefore discolor or alter the general appearance of the surface to which it is applied; and is not harmful or deleterious to the fabric to which it is applied.

In order to enable others to understand, prepare and apply my improved composition, I will now proceed to describe the same 35 in detail giving what I have discovered to be the relative proportions of the ingredients for compounding the mixture. In stating the relative proportions of the ingredients, it will be observed that no absolutely fixed relation exists between the same, but that the proportions of the various ingredients may be changed within certain 40 limits hereinafter stated, the proportions being varied to suit the particular kind of 45 fabric or material to be treated.

The formula is as follows: ten to fifteen parts of pure rubber cement, four and one-half to seven parts of spirits of turpentine, two to four parts of refined paraffin wax, 50 twenty to forty parts of gasoline, and forty to seventy-five parts of tetrachlorid of carbon.

The ingredients above named, after selecting relative parts of the same within the 55 limits mentioned, are thoroughly mixed and agitated until the particles are fully broken

up. The gasoline and tetrachlorid of carbon serve as vehicles for the ingredients suspended therein and form a free flowing composition which may be readily applied as a thin coating and which will readily adhere to and permeate the fabric or material to be coated. However, as some of the ingredients are inflammable substances which will readily catch fire, and especially gasoline, tetrachlorid of carbon is added to the mixture which so changes the inflammable properties thereof that my composition, or the fabric or material coated therewith, will not readily catch fire. It will be noted that a substantial part of the composition is composed of tetrachlorid of carbon (40 to 75 parts being used) and that the proportion of tetrachlorid of carbon is equal or greater than that of the gasoline whereby to insure 75 the noninflammability of the composition and the coated fabric.

The formula given is satisfactory and practical, but I do not consider the invention restricted to the employment of all the specific ingredients above named, the essential feature of the invention being the employment of the tetrachlorid of carbon; the other ingredients may be substituted by their equivalents in the composition, and in some instances for some uses the paraffin wax, or the gasoline or both might be omitted; and while I have referred to "gasoline" in the formula, another equivalent light hydrocarbon might be employed.

What I claim is:

1. A water-proofing composition, comprising a mixture of dissolved rubber and tetrachlorid of carbon, the proportion of tetrachlorid of carbon being at least equal to that of the solvent in the dissolved rubber, to render the composition and fabric coated therewith noninflammable, substantially as described.

2. A noninflammable water-proofing composition, comprising a mixture of rubber cement, spirits of turpentine, paraffin wax, gasoline, and tetrachlorid of carbon, the proportion of tetrachlorid of carbon being at least equal to that of the solvent, to render the composition and fabric coated therewith noninflammable, substantially as described.

3. A composition of matter, comprising a mixture of rubber cement, spirits of turpentine, gasoline and tetrachlorid of carbon, in substantially the following proportions: 10 to 15 parts of rubber cement, 4½ to 7

parts of spirits of turpentine, 20 to 40 parts of gasolene, and 40 to 75 parts tetrachlorid of carbon, substantially as described.

4. The herein-described composition, comprising a mixture of 10 to 15 parts of rubber cement,  $4\frac{1}{2}$  to 7 parts of spirits of turpentine, 20 to 40 parts gasolene, and 40 to 75 parts tetrachlorid of carbon, the physical characteristics of which are that it is noninflammable and water-proof, substantially as described.

5. A composition of matter, comprising a mixture of rubber cement, spirits of turpentine, paraffin wax, gasolene and tetrachlorid 15 of carbon, in substantially the following proportions: 10 to 15 parts of rubber cement,  $4\frac{1}{2}$  to 7 parts of spirits of turpentine, 2 to 4 parts paraffin wax, 20 to 40 parts of gasolene, and 40 to 75 parts tetrachlorid of carbon, substantially as described.

6. The herein-described composition, comprising a mixture of 10 to 15 parts of rubber cement,  $4\frac{1}{2}$  to 7 parts of spirits of turpentine, 2 to 4 parts of paraffin wax, 20 to 40 parts gasolene, and 40 to 75 parts tetrachlorid of carbon, the physical characteris-

tics of which are that it is noninflammable and water-proof, substantially as described.

7. A non-inflammable water-proofing composition comprising a mixture of rubber cement, gasolene and tetrachlorid of carbon in substantially the proportions specified.

8. A non-inflammable water-proofing composition comprising a mixture of rubber cement, spirits of turpentine, gasolene and 35 tetrachlorid of carbon in substantially the proportions specified.

9. A non-inflammable water-proofing composition comprising a mixture of rubber cement, spirits of turpentine, paraffin wax, 40 gasolene, and tetrachlorid of carbon in substantially the proportions specified.

10. A non-inflammable water-proofing composition comprising a mixture of substantially the following proportions: 10 to 45 15 parts of rubber, 20 to 40 parts of a light liquid hydro-carbon, 40 to 75 parts tetrachlorid of carbon, and  $4\frac{1}{2}$  to 7 parts of another solvent, substantially as described.

In testimony that I claim the foregoing 50 as my own, I affix my signature.

JAMES O. PERSONS.